

## UNITED STATES PATENT OFFICE.

FELIX VISINTAINER, OF NEW YORK, N. Y.

## ALLOY.

No Drawing.

Application filed June 2, 1926. Serial No. 113,334.

This invention relates to metallic alloys and in particular to an improved alloy adapted for general use where hardness is a requisite.

5 A particular object of the invention is to provide a new and improved alloy which is non-corrosive and will not rust, which is acid-resistant, which will retain its luster and which is of extreme hardness and one 10 which is capable of withstanding great stresses and severe and sudden shocks.

A further object of the invention is to produce an alloy characterized by its great tensile strength and homogeneity of structure as well as one that may be used in the place of nickel plating which will take a high polish and retain the polish without the necessity of machining.

The alloy in its preferred composition 20 consists of a mixture of the following ingredients in approximately the proportions specified, namely:

|             | Per cent |
|-------------|----------|
| Copper      | 87.05    |
| 25 Aluminum | 11.80    |
| Iron        | 0.43     |
| Silicon     | 0.49     |
| Tin         | 0.10     |

Although I prefer to make the improved 30 alloy from the various ingredients in the proportions given above for the best results, not only as to the heat and acid resisting qualities of the alloy, its homogeneity of structure, and its great compressive strength 35 and ability to withstand shocks, but also as to the adaptability of the alloy for casting and other forming operations, nevertheless, I have found that an alloy, satisfactory 40 for the purposes of the invention and having substantially the qualities obtained by compounding the ingredients in the quantities hereinbefore referred to, may be made from these various ingredients within the following limits:—

|          | Per cent         |
|----------|------------------|
| Copper   | about 85 to 89   |
| Aluminum | about 9 to 13    |
| Iron     | about .25 to .65 |
| Silicon  | about .30 to .70 |
| 50 Tin   | about .07 to .12 |

The ingredients are melted together to form the alloy which can be poured while molten into molds in which it is cast into the desired form. The resultant product is one of high color and brilliant luster and 55 extreme hardness and the surfaces of the article formed therefrom may be polished in any well-known or preferred manner and, as the result of the polishing operation and without the necessity of depositing any 60 coating or plating thereon, the article has imparted thereto a high luster, which it will retain without tendency to tarnish.

The alloy is of extreme hardness and in laboratory tests using the Brinnell method 65 for hardness, the alloy is given a rating of 266 in the Brinnell hardness test.

For compression, a piece of the alloy measuring 1.003 x 0.991 inches having the height 70 of 2.05 inches was subjected to a load of 100,000 pounds with the result that the distortion was found to be 1.015 inches by 0.995 inches or a distortion only measurable in the thousandths of an inch, which is not appreciable in test pieces of larger dimensions.

It will therefore be noted that this alloy will stand an enormous pressure per square inch without breaking down or displaying 80 evidences of brittleness, which is usually present in very hard metallic alloys.

It will be evident, therefore, that I have provided an improved alloy which is non-corrosive, rust-proof, acid resistant and is of extreme hardness and also possesses 85 highly desirable properties and capable of many uses. It should be manifest that a considerable range in proportions of the various ingredients may be invoked within the scope of my invention as defined in the 90 following claims.

What I claim is:

1. An alloy consisting of the following ingredients in substantially the proportions specified: copper 85 to 89%; aluminum 9 95 to 13%; iron .25 to .65%; silicon .30 to .70%; tin .07 to .12%.

2. An alloy of extreme hardness consisting of the following ingredients in substantially the proportions specified: copper 85 100

to 89%; aluminum 9 to 13%; iron .25 to .65%; silicon .30 to .70%. ingredients in substantially the proportions specified: copper 87.05%; aluminum 11.80%; iron .43% and silicon .49%. 10

3. An alloy consisting of the following ingredients in the proportions specified: In testimony whereof I affix my signature.

5 copper 87.05%; aluminum 11.80%; iron .43%; silicon .49%; and tin .10%.

4. An alloy consisting of the following

FELIX VISINTAINER. [L. s.]